

March 29, 1932.

E. P. MULLAN

1,851,369

PROCESS FOR THE PRODUCTION OF NEGATIVES WITHOUT PHOTOGRAPHY

Filed Jan. 29, 1930



CROSS SECTIONS OF NEGATIVE-MAKING STEPS



INVENTOR

By *Edward P. Mullan*  
*W. Williamson* *Atty.*

## UNITED STATES PATENT OFFICE

EDWARD P. MULLAN, OF BALA, PENNSYLVANIA

## PROCESS FOR THE PRODUCTION OF NEGATIVES WITHOUT PHOTOGRAPHY

Application filed January 29, 1930. Serial No. 424,452.

My invention relates to new and useful improvements in a process for the production of negatives without photography, and has for its object the production of negatives from 5 lithographic, steel, copper or other intaglio engravings, half-tones, line cuts, wood cuts, and all other relief plates, lithographic drawings in line, stipple, Ben Day or crayon and all drawings made by any planographic processes, without the use of photographic plates, either wet or dry, films, cameras, printing frames or other photographic equipment.

Fig. 1 is a view of a sheet of material or base having one surface covered with a dextrene coating constituting the first step of the comprehensive process, one corner of the base being left uncovered for illustrative purposes.

Fig. 2 is a view showing the second step wherein the dextrene coating is covered with a 20 collodion coating.

Fig. 3 is a view illustrating the third step of the process wherein an impression is pulled on the collodion coating.

Fig. 4 is a view of the fourth step during 25 which the light resisting background is applied.

Fig. 5 is a view illustrating the fifth step at which time the impression is reversed by removal of the substance forming the impression.

Fig. 6 is a view showing the sixth step of the process wherein a rubber coating is applied. This view illustrates said rubber coating, in particular, between the uncovered part 30 of the background and the balance thereof which is visible through the rubber coating.

Fig. 7 is a view showing, in a manner similar to Fig. 6, the seventh step wherein the rubber coating is covered with a collodion 40 coating.

Fig. 8 is a view of the next step during which the original base is removed.

Fig. 9 is a view illustrating the final step at which time the negative is mounted upon 45 a transparent permanent base or protective backing.

Figs. 10 to 18 inclusive, are exaggerated cross sections of Figs. 1 to 9 inclusive, respectively.

50 In carrying out the process, I first provide

gummed paper which may be any soft paper, preferably unsized, coated with a dextrin solution. The dextrin solution is made by boiling dextrin in water. A flat dextrin solution is preferred and is applied to the paper in the 55 form of a thin paste.

This gummed or dextrin coated paper is next coated on the gummed side with a collodion solution composed of ether, alcohol and negative cotton in the proportions of one 60 pint of ether, one pint of alcohol and one hundred and ninety-two grains of negative cotton.

After the collodion coating is thoroughly dried, an impression is pulled upon the coated 65 surface using ordinary printing or transfer ink and the paper under ordinary conditions can be used in a dry state but when the impression is to be pulled from an intaglio engraving, said paper should be softened by 70 laying between damp blotters or damp unsized news stock.

The impression thus obtained is then reversed by spraying or flowing any opaque 75 solution upon the paper and when said solution is dried, the ink lines are removed with a wad of soft cotton soaked in benzol. The opaque solution may be india ink, black or colored dyes of red, brown or orange shades.

In order to obtain the best or excellent results, said solution should be sprayed with an air brush. The lines which were black on a white background or field now are reversed and appear white on a black background or field. This unfinished negative is now flowed 80 with a rubber solution in the proportions of one-half ounce of pure Pará rubber dissolved in sixteen ounces of benzine. The rubber should be shredded so that it will dissolve easily and quickly. When the rubber solution 85

has dried, the unfinished negative is then flowed with a solution of alcohol, ether, cotton and castor oil produced in the proportions of one pint of alcohol, one pint of ether, ninety-six grains of negative cotton and three 90 minums of castor oil.

After the last mentioned solution has dried, the print is placed in a bath of five per cent acetic acid and the film which has been produced becomes detached from its paper sup- 100

port and can be readily stripped or mounted upon glass, celluloid or any other transparent support.

Where an opaque background is desired, 5 this may be produced by adding to the first coating solution of ammonium iodide and cadmium bromide in the proportions of five grains of ammonium iodide and one grain of cadmium bromide to each ounce of the first 10 coating solution.

A print is made on this coating in the manner described and is then flowed with a solution composed of nitrate of silver distilled water and made slightly acid by the use of 15 chemically pure nitric acid in the proportions of forty-five grains of nitrate of silver dissolved in an ounce of distilled water with a few drops of chemically pure nitric acid. The nitrate of silver solution is allowed to stand 20 on the print for a short time, say approximately two minutes after which the print is developed in a solution of ferrous sulphate, acetic acid, alcohol and water in approximately 25 the proportions of sixteen ounces of water, one ounce of ferrous sulphate, one ounce of acetic acid and one ounce of alcohol. This solution should be filtered and kept cool for use from time to time.

After the background is developed to sufficient intensity, the ink image is removed by 30 soaking with benzol and the print then fixed in a solution of cyanide of potassium in approximately the proportions of one ounce of cyanide of potassium to twenty-four ounces 35 of water. After fixing, the film is removed from the paper support and stripped upon the transparent support in the manner hereinbefore described.

Having thus fully described my invention, 40 what I claim as new and useful is:—

1. The process for the production of negatives without photography consisting in coating soft paper with a dextrin solution; then 45 coating the gummed side of said paper with a solution of ether, alcohol and negative cotton, then pulling an impression upon the coated surface through the medium of ordinary printing and transfer ink; then reversing the impression by applying an opaque 50 solution to the paper; then removing the ink lines by the application of benzol on a wad of soft cotton, then flowing the negative with a solution of rubber dissolved in benzine; when dried, flowing the negative with a solution 55 of alcohol, ether, negative cotton and castor oil; when again dried, placing the print in a bath of five per cent acetic acid to detach the produced film from the paper after which said film may be stripped upon a transparent 60 support.

2. The process for the production of negatives without photography consisting in coating the gummed side of dextrin coated soft paper with a solution of ether, alcohol and negative cotton in the proportions of one pint 65

of ether, one pint of alcohol and one hundred and ninety-two grains of negative cotton, then pulling an impression upon the coated surface by the use of ordinary printing or transfer ink, then reversing the impression by applying an opaque solution to the paper; then removing the ink lines; then flowing the negative with a solution of rubber and benzine in the proportions of one-half ounce of pure Pará rubber dissolved in sixteen ounces of benzine; then drying the negative; then flowing the negative with a solution of alcohol, ether, negative cotton and castor oil in the proportions of one pint of alcohol, one pint of ether, ninety-six grains of negative cotton 80 and three miniums of castor oil, then again drying the negative; then placing the same in a five per cent acetic acid bath to detach the produced film from the paper after which said film may be stripped upon a transparent support.

3. A process for the production of negatives without photography, consisting of coating a base with a transparent film, said base being of a character to permit the removal 90 of said film, then pulling an impression upon the film, then reversing the impression by applying an opaque solution to the film and removing the impression with a suitable solvent, then coating the film with a solution 95 of rubber, then covering the reversed impression with a transparent film to strengthen and protect the reversed impression, then stripping the completed negative, and then mounting it on a still stronger transparent 100 support.

4. The process for the production of negatives without photography consisting of coating a base with a transparent film insoluble in water, then pulling an impression upon the 105 film, then reversing the impression by applying an opaque solution to the film, then removing the impression, then coating the film with a solution of rubber, then covering the reversed impression with a transparent film 110 to strengthen and protect said reversed impression, then stripping the completed negative, and then mounting said negative on a still stronger transparent support.

5. The process for the production of negatives without photography consisting of coating a base with a transparent film, said base being of a character to permit the removal 115 of said film, then pulling an impression upon the film by the use of a transfer medium, then reversing the impression by applying an opaque solution to the film, then removing the lines produced by the transfer medium, then coating the film with a solution of rubber, then covering the reversed impression with 120 a transparent film, then stripping the completed negative, and then mounting it on a still stronger transparent support.

6. The process for the production of negatives without photography consisting of 130

coating a base with a transparent film insoluble in water, said base being of a character to permit the removal of said film, then pulling an impression upon the film by the use of  
5 ink, then reversing the impression by applying an opaque solution to the film, then removing the ink lines, then coating the film with a solution of rubber, then covering the reversed impression with a transparent film  
10 to strengthen and protect said reversed impression, then stripping the completed negative, and then mounting it on a still stronger transparent support.

7. The process for the production of negatives without photography consisting of pulling an impression on a base covered with a separable light transmitting film by the use of a transfer medium, then reversing the impression by applying an opaque solution to  
15 the film, then removing the lines produced by the transfer medium, then coating the film with a protective solution, then covering the reversed impression with a light transmitting film, then stripping the completed negative,  
20 and then mounting said completed negative on a still stronger light transmitting support.

In testimony whereof, I have hereunto affixed my signature.

EDWARD P. MULLAN.

30

35

40

45

50

55

60